

Aug. 13, 1963

J. M. FRANK ET AL

3,100,677

METHOD OF MAKING REFRACTORY BRICK

Filed July 24, 1959



FIG.1

FIG.2

FIG.3

FIG.4

FIG.5



FIG.6

FIG.7

FIG.8



FIG.9

FIG.10



FIG.11

INVENTOR:  
JOSEPH M. FRANK  
NEIL E. BOYER  
JAMES A. CROOKSTON

By Gravely, Lieder & Woodruff  
ATTORNEYS.

Aug. 13, 1963

J. M. FRANK ET AL

3,100,677

METHOD OF MAKING REFRACTORY BRICK

Filed July 24, 1959

2 Sheets-Sheet 2

FIG.13



FIG.14



FIG.15



INVENTORS.  
JOSEPH M. FRANK  
NEIL E. BOYER  
JAMES A. CROOKSTON

BY

*Gravely, Lieder & Woodruff*  
ATTORNEYS.

1

3,100,677

**METHOD OF MAKING REFRACTORY BRICK**  
Joseph M. Frank, Neil E. Boyer, and James A. Crookston,  
Mexico, Mo., assignors to A. P. Green Fire Brick Com-  
pany, Mexico, Mo., a corporation of Missouri

Filed July 24, 1959, Ser. No. 829,342

5 Claims. (Cl. 18—59)

The present invention relates to a novel method for metal encasing refractory brick for use in the construction of various parts of furnaces, and to a novel metal cased refractory brick made by said method. The brick are widely used in metallurgical furnaces, and, in particular, in the basic open-hearth furnace used for making steel. The brick usually is encased on four sides with the ends uncased, however, less than four sides may be cased and the ends also may be cased.

The purpose of the external plates on the brick is primarily to provide a bonding medium between adjoining brick, which tends to make the furnace structure more resistant to the effect of thermal shock and the attacks of slags and furnace fumes in service. The metal plates tend to oxidize and melt in service, fusing adjoining brick into a more or less monolithic structure on the surface facing the interior of the furnace. At the same time the metal plate further back into the furnace wall retains its integrity, thus providing support to the furnace wall during the life of the furnace structure. The brick without external plates are more subject to thermal shock and to sheeting due to changes in structure resulting from attack by slags and fumes than are brick with external plates.

There are numerous methods used to apply these casings to refractory brick. One method is to press the brick mix into a channel previously inserted into the press cavity, thus forming a metal case on three sides of the brick. The fourth side can then be left free of a metal casing, or a metal casing can be applied through pressure from the upper plunger of the press. In this latter case, the applied metal plate has projections which anchor it to the brick. Another method which is used, is to attach the metal plates to any or all sides of the brick by means of adhesives. Another method is to use a channel of the proper size and to force the channel apart, insert the previously formed brick into the channel, and then to allow the channel to assume its normal position so that it is held to the brick by its spring. This method may be used in conjunction with adhesives.

Another recent method of preparing cased brick is to form a refractory brick in a normal manner and then place two U-shaped channels over the brick from opposite faces in a manner that the legs of the channels overlap. The overlapping legs are then spot welded together to form a brick with a double thickness of metal on each side.

In addition to the external plates described above, it is also common practice to place one or two plates inside the brick. The purpose of this is to provide the brick with even more resistance to the effects of thermal shock and breaking-off or sheeting of the brick in service due to attack by furnace fumes and slags. The internal plates are placed inside the brick in such manner that their long dimensions are perpendicular to the hot-face of the brick as it occurs in service. Thus, the internal plates effectively divide each brick into two or three smaller brick separated by metal plates. By means of these internal plates, the brick are made more resistant to the destructive processes which occur in service than brick having only external plates.

The principal method used to place the internal plates in the brick is an adaptation of the method hereinbefore

2

described for forming the brick into a channel previously inserted into the press cavity. In this instance, a second channel of smaller cross-section but the same length and approximately the same height is placed inside the channel forming the outside casing for the brick. The brick is then pressed, simultaneously forming both the outside metal casing on three sides and the two internal plates. To form a single internal plate, a T-shaped metal form is used in place of the smaller channel. The fourth side can be externally plated as described. Another method which is used to provide the internal plates is to press smaller brick and combine two or three of them into a composite with separating plates to form a full-size brick with both internal and external plates. Another method is to saw a full-size brick into two or three smaller brick and combine these into a composite brick with separating plates to form a full-size brick with internal and external plates. Another recent method is to prefabricate a box of the same external dimensions as the brick which is to be formed. This box is made up of the two side members and the end members but with no top and bottom members. Inside the box one or two plates of similar size to the side members are fastened so as to divide the width of the box into two or three equal parts. The prefabricated metal box thus described is then placed into the press cavity with the open top and bottom placed so that the action of the press will cause the brick mix to be compacted into the box. Thus on pressing, a brick is formed having metal plates on the ends and sides and with one or two internal plates inside the brick. External plates may then be fastened to the remaining two free faces of the brick by means of adhesives or by welding to the other metal faces.

It is an object of the present invention to provide a novel method for forming a refractory brick having its four sides encased with an integral sheet of metal and with the ends uncased.

A further object is to provide a novel method of forming a metal cased refractory brick which includes the steps of inserting the refractory mix in a container and forming the container into a brick of the same perimeter as the container but having less volume, thereby compressing the refractory mix. Another object is to provide a cased refractory brick having a continuous metal casing.

Still another object of the present invention is to provide a method of forming a metal cased refractory brick, having internal plates. Another object is to provide a cased refractory brick having internal plates and a continuous metal casing.

These and other objects and advantages will become apparent hereinafter.

The present invention comprises a process of making cased refractories including the steps of placing a refractory mix into a hollow geometrical shape and forming that shape into the desired refractory brick. The invention further consists in the process hereinafter described and claimed and in the refractory brick made by said process.

FIG. 1 is a perspective view of a sheet before it is formed into the casing for a fire brick,

FIG. 2 is a perspective view of a hollow geometric shape formed in the brick making process,

FIG. 3 is a perspective view of the shape shown in FIG. 2 filled with brick mix and diagrammatically showing a vibratory motion imparted to the filled shape,

FIG. 4 is a perspective view of the shape shown in FIG. 3 with a diagrammatic representation of a brick forming press,

FIG. 5 is a perspective view of a finished brick,

FIG. 6 is a perspective view of a modification of the hollow geometric shape shown in FIG. 2,

FIG. 7 is an end view of a geometric shape containing a spacer,

FIG. 8 is an end view of the brick formed from the shape shown in FIG. 7,

FIG. 9 is an end view of a geometric shape having a modified form of spacer contained therein,

FIG. 10 is an end view of the brick formed from the shape shown in FIG. 9,

FIG. 11 is a perspective view of a brick made of a modified form of casing containing perforations in the outer walls,

FIG. 12 is a partially broken perspective view of a modified spacer plate having perforated flanges,

FIG. 13 is an end view of a geometric shape having another modified form of spacer contained therein,

FIG. 14 is an end view of the brick formed from the shape shown in FIG. 13, and

FIG. 15 is a perspective view of the brick shown in FIG. 14.

A flat sheet or metal plate 10 which preferably is carbon steel or a similar oxidizable metal and is of any predetermined length and width (FIG. 1) is conventionally rolled and the opposite edges joined into a hollow geometric shape 11 (FIG. 2) which has an infinite number of possible dimensions for length, width and height. The hollow geometric shape is formed into the predetermined cross-section of established perimeter and shape by usual sheet-metal forming techniques and joined to form a continuous cross-section. The cross-section of the hollow shape is shown as circular in FIG. 2 and elliptical in FIG. 6 and can be any suitable cross-section having a perimeter substantially equal to the perimeter of the refractory brick. The important consideration is that the perimeter of the cross-section of the shape be substantially equal to the perimeter of the cross-section of the shape to which it will be transformed in the brick-forming operation. The metal case may stretch slightly in the brick-forming process if a sufficient amount of refractory mix is placed in the geometrical shape before it is formed into a brick. However, the perimeter of the final brick is substantially the same as the perimeter of the hollow geometrical shape in all cases. In addition, it is an essential feature of the present invention that the area of the cross-section of the hollow geometric shape be greater than the area of the cross-section of the shape to which it will be transformed in the brick-forming operation. This allows rigid control over the density of the final brick. The end joint of the metal sheet 10 can be overlapped as shown in FIG. 2 to form a seam 11a, or it can be butt welded, if desired.

Following the fabrication of the hollow geometric shape 11 from the metal sheet 10 (FIG. 2), it is filled (FIG. 3) with a predetermined amount of a refractory brick mix 12. The refractory can be any known refractory, but is preferably a basic refractory. The amount of brick mix to be placed into the shape may be measured by weight or by volume with similar final results. In addition to merely filling the shape with brick mix it is necessary to compact it by means of vibration, pressure, or a combination of these two mechanisms. The vibratory compacting step is diagrammatically indicated by the arrows "A" in FIG. 3. The necessity for compaction is two-fold—one, to give a final brick of required density, and two, to achieve a degree of compaction or stability of the brick mix in the geometric shape to allow the assembly to be handled with a minimum of loss of brick mix.

The hollow geometric shape 11 which has been filled and compacted with brick mix 12 is then introduced to a brick-forming press (diagrammatically indicated by the arrows 13 in FIG. 4), where the original geometric shape 11 is transformed into the final brick form 14 (FIG. 5). The brick 14 includes a refractory portion 12 and a metal

case 15 having sides 16 and free ends 17. The ends 17 can be left open or can have metal caps or plates attached thereto as by welding or gluing. Since the perimeter of the cross-section of the original geometric shape 11 is substantially equal to the perimeter of the cross-section of the final brick 14, and the area of the cross-section of the original geometric shape 11 is greater than the area of the cross-section of the final brick 14, a brick 14 is formed of the required volume and density with a continuous metal casing 15 on four sides 16. The refractory part 12 of the brick 14 has a greater density since the cross-sectional area and consequently the volume of the metal casing 15 is reduced in the brick-forming process. The metal case 15 retains the refractory portion 12 of the brick 14 by the stresses set up in the brick-forming process, and cannot be removed without the destruction of the brick.

The process may be modified to allow the incorporation of internal steel plates 20 in the final brick 14 (FIGS. 7-10). The plates 20 are introduced into the hollow geometric shape 11 prior to filling it with brick mix 12. The shape of the internal plates 20 can vary, two possibilities being illustrated in FIG. 7 and FIG. 9. As can be seen, FIG. 7 shows the internal plates 20 formed in the shape of a cross, while FIG. 9 illustrates the use of plates 20 in the form of an X. Other possible designs include the use of a concentric circle in the original hollow geometric shape, which on final transformation in the pressing operation becomes a small rectangle within a larger rectangle. Another possibility is shown in FIGS. 13-15 and comprises a corrugated or S shaped plate 30 positioned in the hollow geometric shape 31 so that the final brick forming pressure will act to reduce the distance between corrugations and increase the height of the corrugations. Any design may be used for the internal plates, so long as the plates when introduced into the hollow geometric shape are not longer or wider than the corresponding final brick dimensions. From these examples, it is apparent that many designs not specifically mentioned in this description could be used which would not, however, depart from the spirit and scope of this invention.

A modification of this invention shown in FIG. 11 is to use steel plate which is perforated rather than solid to form the hollow geometric shapes. This produces a brick 14 including a refractory portion 12 and a metal casing 15 having sides 16 with perforations 21 provided therein.

Expanded metal can also be used to form the outer metal casing for the brick, and the term perforated is intended to include such casing constructions.

FIG. 12 shows a modified spacer plate 25 provided with perforations 26 in the flange portions 27. This spacer plate also may be made from expanded metal. Either the solid or perforated form of the spacer can be used with all types of casings and refractory mixes.

By the use of perforated sheet steel or expanded metal as the casing and for the internal plates, a reduction in weight of the final brick is effected while at the same time providing the same support to the furnace structure as is provided with non-perforated sheet steel. In addition, if the internal plates have perforations in them, the density of the refractory mix will be more uniform since it can flow through the openings in the plates from one compartment to another. The use of non-solid casings and internal plates results in more brick units being available per ton of refractory than if solid casings and plates are used.

Thus it is seen that the present invention provides a refractory brick and a method of preparing same which achieves all of the objects and advantages sought therefor. The present invention further provides a brick having an integral or continuous metal casing on four sides thereof, said casing being formed around the brick during the brick making process so that it becomes in effect an

integral part with the brick, tightly adhering, and resisting any attempt at removal without destruction of the metal case.

By reducing the volume of a given geometric shape without substantially changing the perimeter of the cross-section from that of the original shape, it is possible to control the density of the final brick within close limits, and to achieve a very high density in the brick.

The design of the internal plates in the brick can be varied, and the internal plates also are an integral part 10 of the brick.

As indicated, the metal casings and spacers are usually made of low carbon steel, although they can be any ordinary metal or alloy, preferably one which is oxidizable at the temperature encountered in the installation. Stainless steel can also be used.

The brick mix used is preferably a basic refractory type such as dead burned magnesite or chrome ore or mixtures of chrome ore and magnesia. Any suitable basic refractory mix may be used.

A binder should be utilized in the brick mix to enable the brick to hold together without kiln firing. Binders such as dextrin, gum arabic, sulphite pitch, magnesium sulphate, magnesium chloride, sodium dichromate, sodium silicate, etc. are suitable in amounts up to about 5% by weight of the brick mix.

A further variation of this invention is to use a hollow geometric shape, the perimeter of whose cross-section is only slightly smaller than the perimeter of the cross-section of the final brick form or shape. If a sufficient amount of refractory mix is retained in the hollow geometric shape, the final brick-forming operation will act to stretch the metal slightly, resulting in the placement of a residual tensile stress in the metal after the brick is formed, thus providing a more tightly adhering metal case. The perimeter of the final brick is still substantially the same as the perimeter of the hollow geometric shape. The cross-sectional area and the volume of the brick are still reduced from that of the original geometric shape.

This invention is intended to cover all changes and modifications of the examples of the invention herein chosen for purposes of the disclosure, which do not constitute departures from the spirit and scope of the invention.

What is claimed is:

1. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a

60

single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

5. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, placing a spacer plate within the tubular geometrical shape through an open end thereof, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

10. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, placing a spacer plate within the tubular geometrical shape through an open end thereof, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

15. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, placing a spacer plate within the tubular geometrical shape through an open end thereof, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

20. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, placing a spacer plate within the tubular geometrical shape through an open end thereof, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

25. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, placing a spacer plate within the tubular geometrical shape through an open end thereof, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

30. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, placing a spacer plate within the tubular geometrical shape through an open end thereof, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

35. A method of making a metal cased refractory brick adapted to resist the destructive effects of heat consisting of the steps of forming a tubular geometrical shape having a single longitudinal seam, open ends, continuous sides and an established perimeter from a flat sheet of oxidizable metal, placing a spacer plate within the tubular geometrical shape through an open end thereof, temporarily closing one end of the tubular shape to effectively prevent loss of refractory material during the subsequent filling operation, filling the tubular geometrical shape with a basic refractory mix through an open end thereof, vibrating said metal shape along its length to partially compact the refractory mix within the shape to a sufficient extent to cause it to be self-supporting therein, placing the filled tube into a mold housing side and end walls of the final desired form and in a single compression step applying pressure to the outer surface of said metal shape along its length in a direction perpendicular to the direction of vibration and forming the refractory filled geometrical shape into a metal cased refractory brick having only one fabrication seam in the casing and having uncased ends, said brick being of substantially the same perimeter as and of a smaller cross-sectional area and smaller volume than the original geometric shape, said refractory brick having uncased ends and a tightly packed body with a smooth continuous metal casing integrally associated therewith.

3. The method defined in claim 2 wherein said spacer 40 has a + shape.

4. The method defined in claim 2 wherein said spacer has an X shape.

5. The method defined in claim 2 wherein said spacer is corrugated and has an S shape.

45

References Cited in the file of this patent

UNITED STATES PATENTS

|    |           |             |       |               |
|----|-----------|-------------|-------|---------------|
| 50 | 1,406,542 | Crocker     | ----- | Feb. 14, 1922 |
|    | 1,571,087 | Jackson     | ----- | Mar. 18, 1930 |
|    | 1,760,861 | Parker      | ----- | May 27, 1930  |
|    | 1,846,290 | Walter      | ----- | Feb. 23, 1932 |
|    | 2,216,813 | Goldschmidt | ----- | Oct. 8, 1940  |
| 55 | 2,247,376 | Heuer       | ----- | July 1, 1941  |
|    | 2,622,314 | Bergan      | ----- | Dec. 23, 1952 |
|    | 2,673,373 | Heuer       | ----- | Mar. 30, 1954 |
|    | 2,747,231 | Reinhardt   | ----- | May 29, 1956  |
|    | 2,759,256 | Bergan      | ----- | Aug. 21, 1956 |
| 60 | 2,791,116 | Heuer       | ----- | May 7, 1957   |